

# United States Patent Office

2,925,400

Patented Feb. 16, 1960

1

2,925,400

## POLY- $\alpha$ -OLEFINS STABILIZED WITH LONG CHAIN ALKYL GALLATES

Clarence E. Tholstrup and Alan Bell, Kingsport, Tenn., assignors to Eastman Kodak Company, Rochester, N.Y., a corporation of New Jersey

No Drawing. Application October 18, 1957  
Serial No. 690,890

10 Claims. (Cl. 260—45.85)

This invention relates to the stabilization of organic compounds which are subject to oxidative degradation, through the inclusion of certain long chain alkyl esters of gallic acid. More particularly it concerns the addition of low concentrations of certain particular alkyl esters of gallic acid, wherein the alkyl group contains 12-18 carbon atoms, in organic plastic compositions comprising polymerized  $\alpha$ -monoolefins.

It has been demonstrated previously that esters of gallic acid can be used to achieve favorable results as antioxidants with fats, oils, and fatty food products, either when used alone or in a synergistic capacity. Considerable preference has been shown, however, for the antioxidant action of the short chain alkyl gallates, those skilled in the art believing that long chain alkyl radicals would not enhance the antioxidant characteristics of the gallic moiety due to steric effects. Moreover, reduced antioxidant potency per unit of molecular weight would be expected for the higher alkyl gallates. Also, lower alkyl gallates such as ethyl or propyl gallate have been used to stabilize polymeric compositions such as polyethylene. It would be an obvious expectation that, when tested on an equal weight basis, the potency of the gallate compounds would tend to decrease as the ester group increases to fairly large size and weight. Thus, it would be supposed that as the alkyl moiety becomes larger, the active antioxidant gallic moiety would become smaller in proportion, resulting in a commensurate decrease in the relative antioxidant capability of the compound. For example, in the propyl gallate molecule, the active gallic moiety comprises about 80% of the weight of the molecule; whereas, in dodecyl gallate the active gallic moiety comprises only about 50% of the molecule. Long chain alkyl gallates, such as lauryl gallate, have been suggested as antioxidants for foods containing fatty constituents whereby there is achieved a high degree of compatibility even though the presence of the lauryl or similar large alkyl radical obviously diminishes the proportion of the active gallic moiety in inverse relation to the size of such alkyl radicals. As to the compatibility of propyl gallate in organic plastics such as polyethylene, it is pointed out in prior art such as British Patent No. 618,839 that a wide range of proportions can be employed such as 0.05% to 5% by weight; thus, enhanced compatibility over propyl gallate is obviously not required.

Moreover, butyl gallate and its branched chain isomers normally have substantially no better antioxidant properties than the adjacent propyl homolog. It therefore appears that there would be nothing to gain and much to be lost in trying higher alkyl homologs. Furthermore, the parent compound, gallic acid itself, has shown highly satisfactory results in the other direction, i.e., twice the antioxidant capability of propyl gallate.

With these considerations in mind, it is apparent that to those skilled in the art the present invention is quite unobvious. Thus, it has now been found that certain long chain alkyl esters of gallic acid, more particularly the alkyl esters wherein the alkyl group contains 12-18

2

carbon atoms, are unexpectedly a great number of times more efficacious as stabilizers for the poly- $\alpha$ -monoolefins than the short chain alkyl esters, such as propyl gallate. In fact, the long chain alkyl gallates wherein the alkyl radical contains from 12 to 18 carbon atoms are nearly ten times more effective than propyl gallate in polyethylene at a concentration of 0.01% by weight.

When propyl gallate is added to polyethylene for commercial use in amounts of approximately 0.1% of total composition and the composition is processed at elevated temperatures, such as 150° C., the product in contrast to its normal light color acquires a dark tan or dark brown discoloration. This deficiency places definite limitations on the uses of the final product, especially where a pigment is to be incorporated therein. Quite unexpectedly the present invention does not suffer from this deficiency.

An object of the invention is to provide compositions of matter comprising poly- $\alpha$ -monoolefins containing a stabilizer exhibiting excellent compatibility and substantially no staining or discoloration.

A further object is to provide such compositions of matter containing a stabilizer which is considerably more effective than either gallic acid or various aryl or alkyl esters of gallic acid.

Another object of the present invention is to provide such compositions of matter comprising poly- $\alpha$ -monoolefins in combination with certain long chain alkyl esters of gallic acid wherein the alkyl group contains 12-18 carbon atoms.

Still another object of this invention is to provide the aforementioned compositions wherein the gallic ester stabilizers possess the properties of unusually low volatility, ability to protect such compositions from changes in electrical properties, and increased thermal stability.

Other objects are apparent elsewhere herein. The degree of success attained in these and other important objectives will become further apparent hereinafter.

In accordance with an embodiment of this invention, there is provided a synthetic resinous composition comprising a poly- $\alpha$ -monoolefin in combination with 0.001% to 3% by weight, based on the total weight of the composition, of an alkyl ester of gallic acid wherein the alkyl radical contains 12-18 carbon atoms. These compositions demonstrate a stability against degradation far superior to that which could previously be reasonably expected with the short chain alkyl esters of gallic acid.

Laboratory results obtained using a thermal stability test wherein samples of the stabilized polyethylene composition were stored in a forced air oven in which temperatures such as 160° C. were maintained, show oven lives (expressed in numbers of hours of oven storage before peroxide build-up takes place) which are a great many times longer than when propyl gallate is used at the same concentration. Copending application, Serial No. 685,063 filed September 20, 1957, now Patent No. 2,921,048, by Bell et al. describes in detail this testing procedure. Materials of lower stability than polyethylene, such as polypropylene, were tested at 140° C. rather than the 160° C. temperature used for polyethylene. Experimental evidence makes it clear that polyethylene is not a simple equivalent of polymerized homologs such as propylene, 1-butene, etc. since polyethylene has a much higher inherent stability. Moreover, the other poly- $\alpha$ -monoolefins with which this invention is particularly concerned are isotactic or syndiotactic polymers.

Observations indicate that a particularly outstanding feature of this invention lies in the unexpectedly achieved greater thermal, electrical and oxidative stability. Thus, the stabilized polymers resist damage from changes in electrical properties. Another especially valuable attribute of these stabilized polymers relates to their ex-

ceptional resistance to degradation during extrusion or while otherwise shaping polymers at high temperatures.

Moreover, this invention provides stabilized compositions in which inclusion of the stabilizer does not impart a stain or discoloration to the product. This advantage is especially worthwhile when it is desired to incorporate a pigment. Moreover, inasmuch as the stabilizers as advantageously employed according to this invention do not cause discoloring of the product, the stabilized synthetic resin may be colored in more delicate shades than when a stabilizer causing discoloration is used in amounts required for effective stabilization. Thus, the product is better adaptable for use in the manufacture of containers and wrappers for food and the like. Along with improved non-staining characteristics, the specified long chain alkyl esters of gallic acid are highly compatible with poly- $\alpha$ -olefins, making them easily introduced into an organic plastic composition. Moreover, the esters of our invention display excellent low volatility which is an important advantage, especially in products which are subjected to elevated temperatures or other conditions where the stabilizer may be partially lost.

The poly- $\alpha$ -monoolefins referred to in this invention include polyethylene, polypropylene, polybutene-1, and their copolymers as well as other polymerized  $\alpha$ -monoolefins such as 2,2-dimethylbutene-1.

The high molecular weight esters of gallic acid within the purview of the invention are represented by the following general structure:



wherein R is an alkyl radical of at least 12 carbon atoms and no more than 18 carbon atoms. These gallates can be prepared in accordance with conventional practice. The enumerated examples given below illustrate the remarkable capability evinced by these compounds.

The stabilized poly- $\alpha$ -olefin compositions disclosed therein may be prepared by combining a poly- $\alpha$ -olefin with one of the aforescribed gallic esters, together with any desired modifiers or pigments, on heated rolls in accordance with conventional practice. The composition can be removed from the rolls thereafter. If desired, it can be comminuted by means of a cutter such as a Roll and Jewel cutter. Other means of preparing the stabilized compositions can also be employed, such as mixing in a Banbury mixer or other standard mixing equipment. If desired, the ester can be incorporated with the poly- $\alpha$ -olefin in a solvent which can be removed by subsequent working and seasoning.

The compositions of this invention can include modifiers, plasticizers, lubricants, coloring matter, fillers, or other synthetic or natural resins, in addition to combinations of other stabilizers, antioxidants, and metal deactivators known for retarding the catalytic effect of iron, copper or the like in promoting oxidation. Either colored or colorless products may be produced employing a suitable choice of such materials.

The compositions of this invention can be extruded or molded according to conventional techniques to furnish finished articles in the form of sheets, rods, tubes, films, filaments, nuggets, or any other physical shapes commonly assumed by polyolefinic compositions. An efficacious antioxidant is particularly important during the extrusion of poly- $\alpha$ -monoolefins, such as during film manufacture, for without one, small portions of the polyolefin which remain at the head of the extruder for lengthy periods of time at elevated temperatures decompose into solid obstructions thereby requiring frequent shutdowns to permit cleaning of the extruder.

The invention and its unobviousness is further illustrated but not restricted by the following tables wherein examples show poly- $\alpha$ -monoolefins stabilized with gallic acid and gallic acid esters. These tables clearly show the remarkable results obtained when the alkyl esters have 12-18 carbon atoms in the alkyl radical. The aforementioned thermal stability test was used to obtain the results shown; the percentages of the stabilizer compounds are based on the total weight.

TABLE I

Oven life of polyethylene +0.10% stabilizer measured at 160° C. by described thermal stability test

|    | Stabilizer                                                            | Stability As Hours of Oven Life |
|----|-----------------------------------------------------------------------|---------------------------------|
| 20 | 1. None (Control)                                                     | 2                               |
|    | 2. Short Chain Alkyl Gallates:                                        |                                 |
|    | (a) methyl ester                                                      | 8                               |
|    | (b) propyl ester                                                      | 7                               |
|    | (c) butyl ester                                                       | 8                               |
|    | (d) isobutyl ester                                                    | 7                               |
| 25 | 3. Miscellaneous alkyl and aryl Gallates:                             |                                 |
|    | (a) hexyl ester                                                       | 12                              |
|    | (b) 2-ethylbutyl ester                                                | 15                              |
|    | (c) cyclohexyl ester                                                  | 17                              |
|    | (d) phenyl ester                                                      | 16                              |
|    | (e) octyl ester                                                       | 17                              |
|    | (f) 2-ethylhexyl ester                                                | 17                              |
| 30 | 4. Gallic Acid (not esterified)                                       | 17                              |
|    | 5. Specified Long Chain Alkyl Gallates Included within the Invention: |                                 |
|    | (a) dodecyl ester                                                     | >65                             |
|    | (b) octadecyl ester                                                   | >65                             |

From Table I it is apparent that the miscellaneous esters (alkyl and aryl) encompassed within items 2 and 3 are no better than gallic acid. Moreover, there is not any significant variation of properties among the various alkyl gallates which would indicate that propyl gallate (which has proven commercial adequacy) could be greatly improved upon. Thus, it would appear from items 2, 3 and 4 of this table that in general all esters of gallic acid are substantially equivalent in degree of efficacy. It was therefore quite surprising to find, as clearly demonstrated by item 5 of Table I, that a limited number of long chain alkyl esters possess an entirely different order of stabilizing potency. This represents a remarkable difference in kind in the results achieved.

The results shown in item 5 of Table I are representative of similar results which can be achieved using the 13, 14, 15, 16 and 17 carbon atom homologs as well as the isomers of the 12 and 18 carbon atom alkyl gallates shown in item 5. Such homologs and isomers include tridecyl gallate, tetradecyl gallate, 2-ethyltetradecyl gallate, pentadecyl gallate, hexadecyl gallate, 8-methyl-hexadecyl gallate, heptadecyl gallate, etc.

When the test procedures employed in gathering the results for Table I were repeated using 10 times as much of some of the stabilizers, it was found that the ratios of oven lives for stabilized polyethylene to the control sample were no more than about doubled for propyl gallate, cyclohexyl gallate and gallic acid (none others except dodecyl gallate were tested). In contrast, when 10 times as much dodecyl gallate was used, the achieved oven life ratio remained substantially the same. This demonstrates another unexpected feature of this invention in that the long chain alkyl gallates of the invention can achieve their excellent results at unusually low concentrations whereas a previously known gallate such as propyl gallate even at 1.0% concentration is but little more effective than at 0.1% concentration.

Table II shows the stabilization of isotactic polymers of  $\alpha$ -monoolefins which is similar to the results achieved in regard to stabilizing polyethylene as shown in Table I. Similar results can be achieved as regards other isotactic and syndiotactic polymers such as can be derived from 3-methylbutene-1, pentene-1, 3,3-dimethylbutene-1, 4-

methylpentene-1, 4,4-dimethylpentene-1 and other  $\alpha$ -monoolefins containing from 3 to 8 carbon atoms such as styrene and includes the various copolymers.

TABLE II

*Oven life of polypropylene +0.5% stabilizer measured at 140° C. by described thermal stability test*

| Stabilizer               | Stability As Hours of Oven Life |
|--------------------------|---------------------------------|
| 1. None (Control) -----  | 0.5                             |
| 2. Propyl Gallate -----  | 7.0                             |
| 3. Dodecyl Gallate ----- | 70.0                            |

In addition to the compositions of matter covered by this invention, it also covers the related processes such as a process for stabilizing a solid colorless poly- $\alpha$ -monoolefin against oxidative degradation whereby about 0.001% to 3% by weight of an alkyl ester of gallic acid wherein the alkyl group contains 12-18 carbon atoms is combined at above 140° C. with said poly- $\alpha$ -monoolefin without appreciable staining of said composition, whereby a stabilized solid poly- $\alpha$ -monoolefin is formed characterized by being substantially colorless, retaining its electrical properties during exposure to elevated temperatures for extended periods of time, and being free from loss due to volatilization or separation of said stabilizer at elevated temperatures.

This invention produces especially efficacious and unobvious results at stabilizer concentrations of from 0.01% to 0.05% by weight in polyethylene and from 0.05% to 3% by weight in the other poly- $\alpha$ -monoolefins such as polypropylene, etc. Of course, higher quantities can be used in both cases, but generally there is relatively little additional advantage to be gained thereby. A very valuable attribute of the stabilizers of this invention in polyethylene is that they serve quite effectively at concentrations such as 0.05% by weight; whereas, even 1.0% of propyl gallate only improves the AOM stability by a factor on the order of 2 to 4 times and concentrations as low as 0.05% are practically ineffective. In contrast, the small amount of 0.1% of dodecyl gallate results in an improvement factor on the order of more than 30 times (see Table I) and less than half this concentration (lower than 0.05%) is still highly effective. In fact, it is generally quite feasible to employ 0.05% by weight of the stabilizers of this invention as an effective concentration in polyethylene of standard commercial quality.

Although the invention has been described in considerable detail with reference to certain preferred embodiments thereof, it will be understood that variations and modifications can be effected without departing from the spirit and scope of the invention as described hereinabove and as defined in the appended claims.

We claim:

1. A solid polymer of an  $\alpha$ -monoolefin selected from the group consisting of polyethylene, substantially isotactic polymers of  $\alpha$ -monoolefins containing from 3 to 8 carbon atoms and substantially syndiotactic polymers

of  $\alpha$ -monoolefins containing from 3 to 8 carbon atoms stabilized with about 0.001% to 3% by weight, based on total weight of composition, of an alkyl ester of gallic acid wherein the alkyl group contains 12-18 carbon atoms.

2. Solid polyethylene stabilized with an alkyl ester of gallic acid wherein the alkyl group contains 12-18 carbon atoms.

3. Substantially isotactic polypropylene in an essentially solid state stabilized with an alkyl ester of gallic acid wherein the alkyl group contains 12-18 carbon atoms.

4. Polyethylene in an essentially solid state stabilized with about 0.10% by weight, based on total weight of composition, of an alkyl ester of gallic acid wherein the alkyl group contains 12-18 carbon atoms.

5. Polypropylene in an essentially solid state stabilized with about 0.5% by weight, based on total weight of composition, of an alkyl ester of gallic acid wherein the alkyl group contains 12-18 carbon atoms.

6. Polyethylene in an essentially solid state stabilized with about 0.001% to 0.05% by weight of the octadecyl ester of gallic acid.

7. Polyethylene in an essentially solid state stabilized with about 0.001% to 0.05% by weight of the dodecyl ester of gallic acid.

8. Polypropylene in an essentially solid state stabilized with about 0.05% to 3.0% by weight of the dodecyl ester of gallic acid.

9. Polypropylene in an essentially solid state stabilized with about 0.05% to 3.0% by weight of the octadecyl ester of gallic acid.

10. A process for stabilizing a solid colorless poly- $\alpha$ -monoolefin against oxidative degradation whereby about 0.001% to 3% by weight, of an alkyl ester of gallic acid wherein the alkyl group contains 12-18 carbon atoms is combined at above 140° C. with said poly- $\alpha$ -monoolefin without appreciable staining of said composition, whereby a stabilized solid poly- $\alpha$ -monoolefin is formed characterized by being substantially colorless, retaining its electrical properties during exposure to elevated temperatures for extended periods of time, and being free from loss due to volatilization or separation of said stabilizer at elevated temperatures, said poly- $\alpha$ -monoolefin being selected from the group consisting of polyethylene, substantially isotactic polymers of  $\alpha$ -monoolefins containing from 3 to 8 carbon atoms and substantially syndiotactic polymers of  $\alpha$ -monoolefins containing from 3 to 8 carbon atoms.

11. A process for stabilizing a solid colorless poly- $\alpha$ -monoolefin against oxidative degradation whereby about 0.001% to 3% by weight, of an alkyl ester of gallic acid wherein the alkyl group contains 12-18 carbon atoms is combined at above 140° C. with said poly- $\alpha$ -monoolefin without appreciable staining of said composition, whereby a stabilized solid poly- $\alpha$ -monoolefin is formed characterized by being substantially colorless, retaining its electrical properties during exposure to elevated temperatures for extended periods of time, and being free from loss due to volatilization or separation of said stabilizer at elevated temperatures, said poly- $\alpha$ -monoolefin being selected from the group consisting of polyethylene, substantially isotactic polymers of  $\alpha$ -monoolefins containing from 3 to 8 carbon atoms and substantially syndiotactic polymers of  $\alpha$ -monoolefins containing from 3 to 8 carbon atoms.

12. A process for stabilizing a solid colorless poly- $\alpha$ -monoolefin against oxidative degradation whereby about 0.001% to 3% by weight, of an alkyl ester of gallic acid wherein the alkyl group contains 12-18 carbon atoms is combined at above 140° C. with said poly- $\alpha$ -monoolefin without appreciable staining of said composition, whereby a stabilized solid poly- $\alpha$ -monoolefin is formed characterized by being substantially colorless, retaining its electrical properties during exposure to elevated temperatures for extended periods of time, and being free from loss due to volatilization or separation of said stabilizer at elevated temperatures, said poly- $\alpha$ -monoolefin being selected from the group consisting of polyethylene, substantially isotactic polymers of  $\alpha$ -monoolefins containing from 3 to 8 carbon atoms and substantially syndiotactic polymers of  $\alpha$ -monoolefins containing from 3 to 8 carbon atoms.

13. A process for stabilizing a solid colorless poly- $\alpha$ -monoolefin against oxidative degradation whereby about 0.001% to 3% by weight, of an alkyl ester of gallic acid wherein the alkyl group contains 12-18 carbon atoms is combined at above 140° C. with said poly- $\alpha$ -monoolefin without appreciable staining of said composition, whereby a stabilized solid poly- $\alpha$ -monoolefin is formed characterized by being substantially colorless, retaining its electrical properties during exposure to elevated temperatures for extended periods of time, and being free from loss due to volatilization or separation of said stabilizer at elevated temperatures, said poly- $\alpha$ -monoolefin being selected from the group consisting of polyethylene, substantially isotactic polymers of  $\alpha$ -monoolefins containing from 3 to 8 carbon atoms and substantially syndiotactic polymers of  $\alpha$ -monoolefins containing from 3 to 8 carbon atoms.

14. A process for stabilizing a solid colorless poly- $\alpha$ -monoolefin against oxidative degradation whereby about 0.001% to 3% by weight, of an alkyl ester of gallic acid wherein the alkyl group contains 12-18 carbon atoms is combined at above 140° C. with said poly- $\alpha$ -monoolefin without appreciable staining of said composition, whereby a stabilized solid poly- $\alpha$ -monoolefin is formed characterized by being substantially colorless, retaining its electrical properties during exposure to elevated temperatures for extended periods of time, and being free from loss due to volatilization or separation of said stabilizer at elevated temperatures, said poly- $\alpha$ -monoolefin being selected from the group consisting of polyethylene, substantially isotactic polymers of  $\alpha$ -monoolefins containing from 3 to 8 carbon atoms and substantially syndiotactic polymers of  $\alpha$ -monoolefins containing from 3 to 8 carbon atoms.

15. A process for stabilizing a solid colorless poly- $\alpha$ -monoolefin against oxidative degradation whereby about 0.001% to 3% by weight, of an alkyl ester of gallic acid wherein the alkyl group contains 12-18 carbon atoms is combined at above 140° C. with said poly- $\alpha$ -monoolefin without appreciable staining of said composition, whereby a stabilized solid poly- $\alpha$ -monoolefin is formed characterized by being substantially colorless, retaining its electrical properties during exposure to elevated temperatures for extended periods of time, and being free from loss due to volatilization or separation of said stabilizer at elevated temperatures, said poly- $\alpha$ -monoolefin being selected from the group consisting of polyethylene, substantially isotactic polymers of  $\alpha$ -monoolefins containing from 3 to 8 carbon atoms and substantially syndiotactic polymers of  $\alpha$ -monoolefins containing from 3 to 8 carbon atoms.

#### References Cited in the file of this patent

#### UNITED STATES PATENTS

2,448,799 Happoldt ----- Sept. 7, 1948

#### FOREIGN PATENTS

618,839 Great Britain ----- Feb. 28, 1949

645,392 Great Britain ----- Nov. 1, 1950

#### OTHER REFERENCES

Bergel: Chemistry and Industry, Apr. 1, 1944, pages 127-128. (Copy in Scientific Library.)